

1

2,866,757

LUBRICANTS CONTAINING DEPOSIT  
CONTROL ADDITIVES

Stanley R. Newman and Robert Y. Heisler, Fishkill, and Norman Alpert, Poughkeepsie, N. Y., assignors to The Texas Company, New York, N. Y., a corporation of Delaware

No Drawing. Application February 24, 1956  
Serial No. 567,435

8 Claims. (Cl. 252—56)

This invention relates to a lubricating oil containing a novel class of additives which act to control deposits in the combustion zone and to minimize the effects of deposits resulting from the combustion of the fuel particularly under low temperature conditions. More specifically, this invention discloses that superior lubricating oils from the standpoint of removal of low temperature deposits, are obtained by addition of a minor amount of polymethylene glycol bis(glycol ether carbonate) of prescribed composition.

As automobile manufacturers annually raise the compression ratio of their engines in the race for higher horsepower, the problem of engine deposits resulting from the fuel becomes increasingly more severe. Engine deposits which find their origin in the fuel are primarily responsible for surface ignition phenomena such as pre-ignition and octane requirement increase (ORI) which is the tendency of spark ignition engines in service to require higher octane fuels for proper performance. There are two avenues by which this problem can be attacked. One approach is through the fuel and the other approach is through the lubricating oil. In our copending application filed of even date, Serial No. 567,445, it is disclosed that superior hydrocarbon fuels from the standpoint of engine deposits result from the incorporation of polymethylene glycol bis(glycol ether carbonates) of prescribed composition. The subject application involves the discovery that the addition of these polymethylene glycol bis(glycol ether carbonates) to a lubricating oil produces a lubricant marked by the ability to maintain a clean engine even with dirty fuels and under low temperature conditions of operation.

In our copending application, Serial No. 567,476 filed of even date, now Patent No. 2,821,539, there are disclosed novel polymethylene glycol carbonates of the general formula



wherein R is a divalent symmetrical polymethylene radical containing at least 4 carbon atoms, R' is an aliphatic hydrocarbon radical containing 1 to 12 carbon atoms and n has a value of 0 to 10. This invention involves the discovery that a particular group of these novel compounds, the polymethylene glycol bis(glycol ether carbonates), are deposit control lubricating oil additives.

The improved lubricating oils of this invention contain a polymethylene glycol bis(glycol ether carbonate) of the general formula



wherein R is a divalent symmetrical polymethylene radical containing at least 4 carbon atoms and preferably 4 to 10 carbon atoms, R' is an aliphatic hydrocarbon radical containing 1 to 12 carbon atoms and n has a value of 1 to 6. The polymethylene glycol bis(glycol ether carbonates) are effective in lubricating oils in concentrations as low as 0.2 volume percent, but concentrations of 0.5 to 3.0 volume percent are normally employed. There

2

is no critical upper limit of concentration, but economic considerations dictate that concentrations less than 5.0 volume percent polymethylene glycol bis(glycol ether carbonate) be present in the lubricating oil.

This invention also contemplates a process for maintaining an internal combustion engine free from deposits, particularly those formed during low temperature operation, by the presence of a polymethylene glycol bis(glycol ether carbonate) in the combustion zone. This can be effected by using a fuel containing polymethylene glycol bis(glycol ether carbonate) as disclosed in the aforescribed co-pending application, by using a lubricant containing a polymethylene glycol bis(glycol ether carbonate) as described herein, by employing a fuel and lubricant both of which contain a polymethylene glycol bis(glycol ether carbonate) or by adding a polymethylene glycol bis(glycol ether carbonate) to either the fuel, lubricant or both during engine operation. In the latter mode of operation, the polymethylene glycol bis(glycol ether carbonate) is added to the gasoline in an amount to constitute 0.01 to 1.0 volume percent of the fuel and/or to the lube to constitute 0.5 to 5 volume percent of the lubricating oil.

The polymethylene glycol bis(glycol ether carbonates) which inhibit the deposit-forming tendencies of hydrocarbon fuels are readily prepared by the series of reactions described in the aforesigned copending application. In general, the preparation involves the formation of a monochloroformate by reaction of phosgene with an ethylene or polyethylene glycol monoalkyl ether and subsequent reaction of the chloroformate with a glycol in the presence of a hydrogen chloride acceptor such as pyridine or quinoline. An alternate reaction procedure involves formation of a polymethylene glycol dichloroformate by reaction of a polymethylene glycol with phosgene and subsequent reaction of the dichloroformate with a monoether of ethylene or polyethylene glycol in the presence of a hydrogen chloride acceptor.

The lubricating oil of this invention is effective in maintaining deposits at a low level with the result that an engine lubricated therewith shows exceptionally clean cylinder head, combustion space, valves and ring belt area. The low deposit level in the engine minimizes surface ignition in all its manifestations, mainly preignition and "knock". In addition, the low deposit level reduces the engine's octane requirement increase. Deposits on surfaces contacted by the additive-containing lubricating oil, such as piston skirts and cylinder walls, are very markedly reduced.

The polymethylene glycol bis(glycol ether carbonates) usable in the lubricants of the invention are exemplified by the following: tetramethylene glycol bis(butoxyethyl carbonate), pentamethylene glycol bis(methoxyethyl carbonate), hexamethylene glycol bis(ethoxyethyl carbonate), hexamethylene glycol bis(propoxymethyl carbonate), pentamethylene glycol bis(butoxyethoxyethyl carbonate), pentamethylene glycol bis(methoxyethoxyethyl carbonate), hexamethylene glycol bis(butoxyethoxyethyl carbonate), pentamethylene glycol bis(methoxyethoxyethyl carbonate), octamethylene glycol bis(ethoxyethyl carbonate), octamethylene glycol bis(methoxyethoxyethyl carbonate), decamethylene glycol bis(ethoxyethoxyethyl carbonate), decamethylene glycol bis(butoxyethoxyethyl carbonate), pentamethylene glycol bis(2-buten-1-oxymethyl carbonate), tetramethylene glycol bis(deoxyethoxyethyl carbonate), tetramethylene glycol bis(ethoxyethoxyethyl carbonate), pentamethylene glycol bis(butoxyethoxyethyl carbonate), pentamethylene glycol bis(ocetoxyethoxyethyl carbonate), pentamethylene glycol bis(pentoxyethyl carbonate), heptamethylene glycol bis(pentoxyethyl carbonate).

It is necessary for the glycol carbonate ester to have the prescribed formula in order to operate effectively as deposit-control additives. If there are more than 6 ethylene oxide units, the additive becomes too water-soluble for proper functioning as a lubricant additive.

The polymethylene glycol bis(glycol ether carbonates) effective in reducing deposit formation in hydrocarbon fuels are all characterized by boiling points above 650° F., a molecular weight above 300 and a carbon to oxygen weight ratio below 2.5. Apparently, the glycol carbonate ester must possess all of these properties simultaneously in order to impart deposit-forming properties to hydrocarbon fuels.

In summary, the following conclusions can be made as to the requirements of each section of the additive molecule for the production of a polymethylene glycol bis(glycol ether carbonate) having deposit-control properties. (1) The polymethylene radical, that is the —R— group contains at least 4 and preferably less than 10 carbon atoms. The ethylene oxide unit, e. g. the —(OCH<sub>2</sub>CH<sub>2</sub>)<sub>n</sub>— group, can contain 1 to 6 units. (2) Two carbonate radicals are required since polymethylene glycol mono carbonate ester derivatives are ineffective as deposit-control additives. (3) Terminal aliphatic radicals contain 1 to 12 carbon atoms with aliphatic radicals containing 2 to 6 carbon atoms being preferred.

The polymethylene glycol bis(glycol ether carbonates) are effective as a deposit-control additive in a concentration of at least 0.2 volume percent of the lubricant. The concentration of the polymethylene glycol bis(glycol ether carbonate) usually falls between 0.5 and 3.0 volume percent of the lubricant. Since the improvement in concentrations higher than 5.0 volume percent is only marginal, a practical upper limit is about 5.0 percent level even though there is no critical upper limit. Economic considerations also dictate that the additive concentration be less than 5 percent.

The polymethylene glycol bis(glycol ether carbonates) of this invention are effective in controlling deposit formation in lubricants employed in spark ignition engines, diesel motors and gas turbines. However, the polymethylene glycol bis(glycol ether carbonates) of prescribed composition are normally used in motor oils for spark ignition engines wherein fuel derived deposits formed during low temperature operation are a particularly vexing problem. Diesel lubricants containing polymethylene glycol bis(glycol ether carbonates) are effective in eliminating deposits resulting from the use of the so-called "economy" diesel fuels, i. e. fuels having a high sulfur content or containing cracked or residual stocks. The polymethylene glycol bis(glycol ether carbonates) are also useful as deposit control additives in gas turbine lubricants which are generally ester base lubricants. The polymethylene glycol bis(glycol ether carbonates) are useful in aviation oils which lubricate reciprocating aviation engines. The scope of the lubricating oils to which the polymethylene glycol bis(glycol ether carbonates) of the invention are added to form superior lubricants is broad and includes mineral oils, synthetic lubricating oils and mixtures thereof.

The hydrocarbon mineral oils usable in this invention can be paraffin base, naphthene base or mixed paraffin-naphthene base distillate or residual oils. Paraffin base distillate lubricating oil fractions are used in the formulation of premium grade motor oils such as are contemplated in this invention. The lubricating base generally has been subjected to solvent refining to improve its lubricity and viscosity temperature relationship as well as solvent dewaxing to remove waxy components and improve the pour of the oil. Broadly speaking, mineral lubricating oils having an SUS viscosity at 100° F. between 50 and 1,000 may be used in the formulation of the improved lubricants of this invention but usually the viscosity range falls between 70 and 300 at 100° F.

The mineral lubricating oils to which the polymethylene glycol bis(glycol ether carbonates) of this invention are added usually contain other additives designed to impart other desirable properties thereto. For example,

5 V. I. improvers such as the polymethacrylates are normally included therein as are materials which act as detergents and dispersants for the removed combustion chamber deposits. The detergent additives, such as basic barium sulfonate and barium alkyl phenolate, provide

10 the required dispersing properties.

The V. I. improver normally used is a polymethacrylate of the general formula



wherein R is an aliphatic radical and n is an integer having a value of more than 1.

The most commonly used detergent-dispersant additive 20 is an alkaline earth metal sulfonate such as calcium petroleum sulfonate or barium petroleum sulfonate. These products are so well known as detergent-dispersant additives they require no further description. Similarly, divalent metal alkyl phenolates are widely used as detergents either alone or in combination with the alkaline earth metal petroleum sulfonates.

The most commonly used inhibitor and antioxidant is 25 a divalent metal alkyl dithiophosphate which results from the neutralization of a P<sub>2</sub>S<sub>5</sub>-alcohol reaction product with a divalent metal or divalent metal oxide. The most widely used inhibitors are barium and zinc alkyl dithiophosphates.

The synthetic lubricating oils are usually of the ester 30 or ether type. High molecular weight, high boiling

35 liquid aliphatic dicarboxylic acid esters possess excellent viscosity-temperature relationships and lubricating properties and are finding ever increasing utilization in lube oils adapted for high and low temperature lubrication; esters of this type are used in the formulation of jet

40 engine oils. Examples of this class of synthetic lubricating bases are the diesters of acids such as sebacic, adipic, azelaic, alkenyl succinic, etc.; specific examples of these diesters are di-2-ethylhexyl sebacate, di-2-ethylhexyl azelate, di-2-ethylhexyl adipate, di-n-amyl sebacate, di-2-

45 ethylhexyl-n-dodecyl succinate, di-2-ethoxy-ethyl sebacate, di-2'-methoxy-2-ethoxyethyl sebacate (the methyl Carbitol diester), di-2'-ethyl-2-n-butoxyethyl sebacate (the 2-ethylbutyl Cellosolve diester), di-2-n-butoxyethyl azelate (the n-butyl Cellosolve diester) and di-2'-n-bu-

50 toxy-2-ethoxyethyl-n-octyl succinate (the n-butyl Carbitol diester).

Polyester lubricants formed by a reaction of an aliphatic dicarboxylic acid of the type previously described, a glycol and a monofunctional aliphatic monohydroxy

55 alcohol or an aliphatic monocarboxylic acid in specified mol ratios are also employed as the synthetic lubricating base in the compositions of this invention; polyesters of this type are described in U. S. 2,628,974. Polyesters formed by reaction of a mixture containing specified

60 amounts of dipropylene glycol, sebacic acid and 2-ethylhexanol and of a mixture containing adipic acid, diethylene glycol and 2-ethylhexanoic acid illustrate this class of synthetic polyester lubricating bases.

Polyalkylene ethers as illustrated by polyglycols are also 65 used as the lubricating base in the compositions of this invention. Polyethylene glycol, polypropylene glycol, polybutylene glycols and mixed polyethylene-polypropylene glycols are examples of this class of synthetic lubricating bases.

70 The sulfur analogs of the above-described diesters, polyesters and polyalkylene ethers are also used in the formulation of the lubricating compositions of this invention. Dithioesters are exemplified by di-2-ethylhexyl thiosebacate and di-n-octyl thioadipate; polyethylene thio-

75 glycol is an example of the sulfur analogs of the poly-

alkylene glycols; sulfur analogs of polyesters are exemplified by the reaction product of adipic acid, thioglycol and 2-ethylhexyl mercaptan.

The action of the polymethylene glycol bis(glycol ether carbonate) in improving the deposit-removing properties of a lubricating oil was demonstrated by a modified Chevrolet deposits test—CRC FL-2-650. The laboratory engines are operated under the standard conditions of this test with the exception that crankcase oil temperatures were 10° F. lower, the water jacket temperatures were 5° F. lower, and the crankcases of the test engines were ventilated. These modifications are in every case in the direction of making the test more severe and are intended to simulate low temperature conditions wherein deposit formation is most pronounced. After the termination of each run, the engine is disassembled and its parts are evaluated by a merit system adapted from the CRC-L-4-1252 test. This merit system involves visual examination of the engine part in question and their rating according to deposits by comparison with standards which have assigned ratings. For example, a rating of 10 on piston skirt designates a perfectly clean piston while a rating of zero represents the worst condition. Similarly, a rating of 100 on total engine deposits represents a perfectly clean engine, etc.

In the following table, there are shown the results obtained in the modified Chevrolet deposits test with lubricating oils containing various concentrations of polymethylene glycol bis(glycol ether carbonates) and of polymethylene glycol bis(alkyl carbonates). Base fuel A used in this test had an 87.0 ASTM research octane rating containing 2.90 ml. of TEL per gallon, had an API gravity of 58.0 and a boiling range between 106 and 396° F.; it was negative in the copper corrosion test and had an oxidation stability in the ASTM test of 530 minutes minimum. Base fuel B had a 90.5 ASTM research octane rating, containing 2.67 ml. of TEL per gallon, had an API gravity of 59.0 and a boiling range between 93 and 395° F.; it was negative in the copper strip corrosion test and had an oxidation stability of 445 minutes minimum. The base fuels also contained minor amounts of gasoline inhibitor, viz., N,N'-di-secondary butyl paraphenylenediamine, lecithin, and N,N'-disalicylidene-1,2-diaminopropane.

The reference lubricating oil was a 20-20W heavy duty oil meeting supplement I requirements. This reference oil contained a methacrylate VI improver and a balanced combination of additives which impart detergent, dispersant and antioxidant properties to the oil. The additive mixtures comprises a barium petroleum sulfonate and a zinc alkyl dithiophosphate in which the alkyl group is a methylcyclohexyl radical.

TABLE I

Engine cleanliness in the modified Chevrolet S-II test

|                                                                  | Piston Skirt | Total Engine Deposits | Concentration of Additive in Oil at Run Termination, Vol. Percent |
|------------------------------------------------------------------|--------------|-----------------------|-------------------------------------------------------------------|
| Base Oil (Fuel A)                                                | 4.7          | 77.7                  | -----                                                             |
| Base Oil (Fuel A) plus:                                          |              |                       |                                                                   |
| 1,5-pentamethylene glycol bis (2-ethoxyethyl carbonate)          | 7.8          | 82.8                  | 3.0                                                               |
| 1,5-pentamethylene glycol bis (2-ethylhexyl carbonate)           | 4.7          | 70.7                  | 3.0                                                               |
| Base Oil (Fuel B)                                                | 6.1          | 79.9                  | -----                                                             |
| Base Oil (Fuel B) plus:                                          |              |                       |                                                                   |
| 1,5-pentamethylene glycol bis (2,2',2"-triethoxyethyl carbonate) | 9.7          | 90.7                  | 2.5                                                               |
| 1,5-pentamethylene glycol bis (n-amyl carbonates)                | 4.8          | 76.8                  | 3.0                                                               |

The data in the foregoing table clearly show that polymethylene glycol bis(glycol ether carbonates) are effec-

tive deposit-control additives for lubricating oils. Ratings above 7.8 in piston skirt deposits and above 80 in total engine deposits are very good results in this low temperature deposits test.

- 5 It is significant that polymethylene glycol bis(alkyl carbonates) which are also disclosed as novel compounds in the aforesaid copending application Serial No. 567,476 are ineffective deposit-control additives. It has been theorized that the ether linkage in the polymethylene glycol bis(glycol ether carbonates) is an important factor 10 in the removal of deposits. Whatever the explanation of the effectiveness of polymethylene glycol bis(glycol ether carbonates) and of the ineffectiveness of polymethylene glycol bis(alkyl carbonates), the results are 15 striking.

Obviously, many modifications and variations of the invention, as hereinbefore set forth, may be made without departing from the spirit and scope thereof and, therefore, only such limitations should be imposed as are indicated in the appended claims.

We claim:

1. A lubricating oil containing a polymethylene glycol bis(glycol ether carbonate) having a carbon to oxygen weight ratio below 2.5 and a boiling point above about 25 650° F. and the general formula



wherein R is a divalent symmetrical polymethylene radical containing at least 4 carbon atoms and preferably 4 to 10 carbon atoms, R' is an aliphatic hydrocarbon radical containing 1 to 12 carbon atoms and n has a value of 1 to 6, in an amount sufficient to eliminate deposits formed during fuel combustion and to maintain a clean engine.

- 35 2. A lubricating oil according to claim 1 containing 0.2 to 5.0 volume percent polymethylene glycol bis(glycol ether carbonate).

3. A lubricating oil according to claim 1 containing 0.5 to 3.0 volume percent polymethylene glycol bis(glycol 40 ether carbonate).

4. A mineral lubricating oil containing a polymethylene glycol bis(glycol ether carbonate) having a carbon to oxygen weight ratio below 2.5 and a boiling point above about 650° F. and the general formula



wherein R is a divalent symmetrical polymethylene radical containing at least 4 carbon atoms and preferably 4 to 10 carbon atoms, R' is an aliphatic hydrocarbon radical containing 1 to 12 carbon atoms and n has a value of 1 to 6, in an amount sufficient to eliminate deposits formed during fuel combustion and to maintain a clean engine.

- 55 5. A lubricating oil according to claim 4 containing 0.2 to 5.0 volume percent polymethylene glycol bis(glycol ether carbonate).

6. A lubricating oil according to claim 4 containing 0.5 to 3.0 volume percent polymethylene glycol bis(glycol 60 ether carbonate).

7. A lubricating oil according to claim 4 containing 0.2 to 5.0 volume percent 1,5-pentamethylene glycol bis(2-ethoxyethyl carbonate).

8. A lubricating oil according to claim 4 containing 0.2 to 5.0 volume percent 1,5-pentamethylene glycol bis(2,2',2" triethoxyethyl carbonate).

#### References Cited in the file of this patent

#### UNITED STATES PATENTS

- 2,370,571 Muskat Feb. 27, 1945  
 2,379,249 Muskat June 26, 1945  
 2,379,250 Muskat June 26, 1945  
 2,379,252 Muskat June 26, 1945  
 2,651,657 Mikeska Sept. 8, 1953